

## UNITED STATES PATENT OFFICE

2,270,400

## FUEL

Joseph A. Wyler, Allentown, Pa., assignor to  
Trojan Powder Company, Allentown, Pa.

No Drawing. Application November 30, 1939,  
Serial No. 306,813

2 Claims. (Cl. 44—9)

This invention relates to fuels in general and more particularly to fuels for Diesel and spark-ignition engines.

An object of my invention is to provide a fuel of shorter delay period when used in high-speed compression engines. By delay period in this type of engine is meant the time interval between the injection and the ignition of the fuel. Another object is to effect a lowering of the compression ratio of the engine. A still further object is to improve the combustion characteristics of fuels generally used in automobile and aeroplane engines. Other and further objects will become apparent upon a perusal of this specification.

I have discovered that the addition of small proportions of tetranitromethane ( $C(NO_2)_4$ ) to oils used in Diesel engines produces a fuel of improved characteristics. In general I may use as much as 5%, by weight, of tetranitromethane in the final mixture, although I prefer about 0.5—1.5%. In a test, using an oil which was already of an especially high quality (cetane number of 68), in an engine which was also of exceptionally high quality (in which the combustion-accelerating reagent would have less chance of showing improvement than it would have in the average compression-ignition engine) compared to the usual compression-ignition engines, it was found that the addition of 4% of tetranitromethane produced a fuel which gave a higher maximum cylinder pressure (without knock) for the same advance angle, an improved exhaust appearance, a general improvement in the combustion of the fuel, a decrease in the ignition lag by 1 crankshaft degree in 10 at 2,000 R. P. M. and permitted four degrees further retardation of injection before misfiring occurred. With an inferior fuel oil to start with these improvements would be more marked, or a lesser amount of tetranitromethane could be used for obtaining the same relative improvement.

5 The solubility and volatility of tetranitromethane are exceptionally favorable for its use not only in the heavier paraffinic oils, but also in the lighter petroleum distillates as kerosene and gasoline. Tetranitromethane dissolves in all proportions in these materials, has a boiling point of about 127° C. and a very favorable vapor tension. It is insoluble in water and, when dry, is non-corrosive to metals.

10 Applicant is aware of the disclosure of such agents as methyl nitrate, ( $CH_3NO_3$ ), ethyl nitrate, butyl nitrate, and the like, for use in improving the ignition characteristics of oils and wishes to emphasize that his agent, tetranitromethane, is a material of an entirely different chemical and molecular constitution and is not in itself an explosive, as are methyl and ethyl nitrates.

15 Although my improved fuel is intended mainly for Diesel engine use, I may use a mixture of gasoline and tetranitromethane, say about 95 parts (by weight) of gasoline to as much as 5 parts (by weight) of tetranitromethane in automotive engines in order to obtain improved combustion characteristics.

20 25 I do not limit myself to the above description except as indicated in the appended claims.

I claim:

30 1. The method of accelerating the ignition of liquid fuels in an internal combustion engine of the type wherein ignition of the fuel is spontaneously effected by injection into the compressed air in the engine cylinder which comprises admixing with the fuel prior to ignition a minor proportion of tetranitromethane.

35 2. The method of accelerating the ignition of liquid fuels in an internal combustion engine of the type wherein ignition of the fuel is spontaneously effected by injection into the compressed air in the engine cylinder which comprises admixing with the fuel prior to ignition about 0.5% of tetranitromethane.

JOSEPH A. WYLER.